

1

2,748,939

PHOSPHATE RECOVERY IN REVERSE FLOTATION  
USING A FLUOSILICATE TO DEACTIVATE THE  
REAGENTSWilliam A. Hedges, Plant City, and Joseph E. Floyd,  
Fort Meade, Fla., assignors to Swift & Company, Chi-  
cago, Ill., a corporation of IllinoisNo Drawing. Application January 24, 1955,  
Serial No. 483,828

15 Claims. (Cl. 209—166)

The present application, which is a continuation-in-part of our earlier application, Serial No. 393,012, filed November 18, 1953, and now abandoned, relates in general to the concentration of phosphate-bearing minerals from their ores, and more specifically to an improvement in the so-called "reverse flotation" method of phosphate recovery.

It has heretofore been proposed, and generally followed in the field of phosphate recovery, to subject the phosphate ore to a concentration step wherein the bulk of the phosphate values is floated in a rougher concentrate along with a minor proportion of silicious gangue, followed by a second concentration step wherein this rougher concentrate is repulped and the silicious gangue floated therefrom. In performing the first step in this process negative-ion reagents, such as the higher fatty acids, are used to selectively coat the phosphate particles, while in the second step positive-ion reagents, such as the higher aliphatic amines, are used to selectively coat the silicious particles. A substantial improvement in the grade and recovery of the final concentrate results when the effect of the negative-ion reagents is removed prior to treatment of the rougher concentrate with the positive-ion reagents. This negative-ion reagent deadening step has heretofore been carried out only by the use of sulfuric acid treatment followed by a washing step, and it has been generally believed that the acid reaction is essential to the removal of the effect of the negative-ion reagents.

It has now been discovered that this is apparently not the case, and that a similar effect may be reproduced without the necessity of using sulfuric acid. The conventional use of sulfuric acid causes an increase in the amount of amine reagent required to float the silica due to the reaction between the amine and the residual acid carried over from the washing step to form an insoluble salt having practically no silica floating power.

It is therefore an object of the present invention to provide a method for deactivating negative-ion reagents in a reverse flotation process for the recovery of phosphatic values wherein sulfuric acid is not required.

It is a further object of the present invention to provide a method for deactivating negative-ion reagents in a reverse flotation process for the recovery of phosphatic values wherein a by-product, produced during the resultant treatment of the phosphatic material, is used.

Additional objects, if not specifically set forth herein, will be readily apparent to one skilled in the art from the following detailed description of the invention.

In accordance with the present invention fluosilicates, such as the metal fluosilicates, including alkali metal and alkaline earth fluosilicates, may be used for deactivating the negative-ion reagents in a reverse flotation process. Obviously, since as stated above, the function of the fluosilicate is to deactivate the negative ion reagent, this fluosilicate must itself be ionizable in water and hence water-soluble. By this term "water-soluble" it is meant that the solubility of the fluosilicate must be sufficient to deactivate the negative ion reagents. In the case of some of

2

these fluosilicates, such as calcium and potassium, the solubility may be only a very small amount. It has been found, for example, that any of the various salts, calcium fluosilicate ( $\text{CaSiF}_6$ ), potassium fluosilicate ( $\text{K}_2\text{SiF}_6$ ), 5 ammonium fluosilicate ( $(\text{NH}_4)_2\text{SiF}_6$ ), magnesium fluosilicate ( $\text{MgSiF}_6$ ), or sodium fluosilicate ( $\text{Na}_2\text{SiF}_6$ ), any of which may be produced from the phosphoric acid made from the recovered phosphatic values, are very effective for use in the invention. These reagents, in quantities 10 as small as one-third the amount by weight of sulphuric acid conventionally required, will produce a similar deactivating of the negative-ion reagents. In addition, the use of these salts does not cause an extensive depression in the pH of the rougher concentrate as does the use of 15 the conventional sulfuric acid and, if carried over from the washings, they do not adversely affect the amine reagent as does the mineral acid. Accordingly, less amine reagent is required to satisfactorily treat a rougher concentrate which has been deactivated with one of these 20 fluosilicates than is required when the deactivation is carried out with sulfuric acid.

The amount of fluosilicate may vary considerably. A sufficient amount to counteract the negative ions will usually range between about 1 and 5 pounds per ton of 25 finished concentrate. The preferred amount is about 2 to 3 pounds.

The deactivators of the present invention, as aforesaid, may be produced as by-products from phosphoric acid which is manufactured from the phosphatic values 30 recovered in the floatation operation. For example, the recovery operation for sodium silico fluoride, which does not form a part of the present invention, comprises adding either sodium hydroxide or a sodium salt, e. g.,  $\text{NaCl}$  or  $\text{Na}_2\text{CO}_3$ , to the phosphoric acid and filtering, washing, 35 and drying the resulting sodium silico fluoride precipitate. While the present invention contemplates primarily the use of fluosilicates obtained from this source and hereinafter referred to as "by-product fluosilicates," it is also within the scope of the present invention to use C. P. 40 fluosilicates and other preparations of such compounds regardless of the source thereof.

The following examples show the effectiveness of the present method under varying conditions as compared with the conventional method using sulfuric acid. These 45 examples are furnished for the purpose of illustration only and are not to be construed as placing any limitation on the scope of the invention other than as appears in the appended claims.

## Example I

50 Silica floats were run on rougher concentrates following deactivation of the negative-ion reagents in such concentrates by the use of sodium silico fluoride in accordance with the present invention. Similar floats were run on rougher concentrates after using the conventional mineral acid deactivation treatment. In both instances the original feeds were approximately identical. The same amounts and types of negative-ion reagents were used in obtaining the rougher concentrates, and the same positive-ion reagent (amine) was used in obtaining the silica float. Under column (a) of the following table are 55 grouped the test data obtained by conditioning a rougher concentrate containing negative-ion reagents at about 60–65 percent solids with 2 pounds  $\text{Na}_2\text{SiF}_6$ /ton of concentrate added. This concentrate was washed twice with clear water to remove the deadened reagents and then subjected to the silica float. The test reported under column (b) was identical to that under column (a) except that the washing step was omitted. A conventional run, using a mineral acid ( $\text{H}_2\text{SO}_4$ ) to deactivate the negative-ion reagent, is reported under column (c) of the following table for comparative purposes. In this run, the rougher concentrate was treated with 6 pounds  $\text{H}_2\text{SO}_4$ /ton 60 65 70

of concentrates, the deadened reagents washed from the concentrate as in test (a), and the silica floated as in the case of the preceding runs.

|                                 | (a)   | (b)   | (c)   |
|---------------------------------|-------|-------|-------|
| Pounds NaOH/ton concentrates    | 0     | 0     | 0.40  |
| Pounds Amine/ton concentrates   | 0.20  | 0.20  | 0.20  |
| Pounds Frother/ton concentrates | 0.20  | 0.20  | 0.20  |
| Percent concentrates            | 86.12 | 92.67 | 86.49 |
| Percent silica froth            | 13.88 | 7.33  | 13.51 |
| B. P. L. feed                   | 69.26 | 68.96 | 68.60 |
| B. P. L. concentrates           | 76.89 | 73.33 | 76.65 |
| B. P. L. silica froth           | 21.98 | 13.79 | 17.11 |
| SiO <sub>2</sub> concentrates   | 1.49  | 6.07  | 1.66  |
| Percent B. P. L. recovery       | 95.58 | 98.55 | 96.64 |

|                                   | (a)   | (b)   | (c)   | (d)   |
|-----------------------------------|-------|-------|-------|-------|
| Percent solids in washing step    | 65.0  | 65.0  | 65.0  | 40.0  |
| pH washing step                   | 5.1   | 5.1   | 5.1   | 3.1   |
| Pounds reagents/ton concentrates: |       |       |       |       |
| H <sub>2</sub> SO <sub>4</sub>    | 0.0   | 0.0   | 0.0   | 6.0   |
| Na <sub>2</sub> SiF <sub>6</sub>  | 2.0   | 2.0   | 2.0   | 0.0   |
| NaOH                              | 0.40  | 0.40  | 0.40  | 0.40  |
| Amine                             | 0.20  | 0.12  | 0.04  | 0.20  |
| Frother                           | 0.20  | 0.12  | 0.04  | 0.20  |
| Percent concentrates              | 80.73 | 82.00 | 85.69 | 55.61 |
| Percent silica froth              | 19.27 | 18.00 | 13.31 | 14.39 |
| B. P. L. feed                     | 67.58 | 67.04 | 66.82 | 67.10 |
| B. P. L. concentrates             | 76.98 | 76.52 | 74.49 | 76.43 |
| B. P. L. silica froth             | 28.23 | 23.85 | 16.87 | 11.58 |
| SiO <sub>2</sub> concentrates     | 1.72  | 1.97  | 4.05  | 2.02  |
| Percent B. P. L. recovered        | 91.93 | 93.63 | 96.67 | 97.52 |

was conducted in the same manner as tests (c) of Examples I and II.

### Example II

Similar tests were run on rougher concentrates containing negative-ion reagents to show the effects of varying the pH of the concentrates in the silica float step and also of reducing the conventional amount of acid to give the same pH in the washing step as that obtained when sodium silico fluoride is used. Under column (a) is reported the results of a test conducted exactly as that reported as (a) in Example I. Test (b) was run exactly the same as test (a) except that caustic soda was added to the concentrate during the silica float. Test (c) was run in the same manner as test (c) of Example I. Test (d) shows the results obtained when the amount of mineral acid is cut down to give substantially the same pH in the washing step as was obtained when sodium silico fluoride was used.

|                                   | (a)   | (b)   | (c)   | (d)   |
|-----------------------------------|-------|-------|-------|-------|
| Percent solids in washing step    | 65.0  | 65.0  | 40.0  | 65.0  |
| pH washing step                   | 6.5   | 6.5   | 3.1   | 6.1   |
| Pounds reagents/ton concentrates: |       |       |       |       |
| H <sub>2</sub> SO <sub>4</sub>    | 0     | 0     | 6.0   | 0.80  |
| Na <sub>2</sub> SiF <sub>6</sub>  | 2.0   | 2.0   | 0.0   | 0.0   |
| NaOH                              | 0.0   | 0.20  | 0.40  | 0.40  |
| Amine                             | 0.20  | 0.20  | 0.20  | 0.20  |
| Frother                           | 0.20  | 0.20  | 0.20  | 0.20  |
| Percent concentrates              | 84.04 | 80.28 | 86.17 | 45.72 |
| Percent silica froth              | 15.96 | 19.72 | 13.83 | 54.23 |
| B. P. L. feed                     | 69.45 | 69.14 | 68.99 | 69.14 |
| B. P. L. concentrates             | 78.27 | 78.58 | 77.99 | 78.23 |
| B. P. L. silica froth             | 23.01 | 30.70 | 12.89 | 61.47 |
| SiO <sub>2</sub> concentrates     | 1.72  | 1.68  | 2.04  | 1.57  |
| Percent B. P. L. recovered        | 94.70 | 93.62 | 97.45 | 51.78 |

### Example III

Similar tests were run on rougher concentrates containing negative-ion reagents to show that good results can be obtained using the deactivator sodium silico fluoride even when the amount of anionic or positive-ion reagent is drastically reduced in the subsequent silica float. Test (a) was run in the same manner as the tests reported as (a) in Examples I and II. Test (b) is the same as (a) except that the amount of positive-ion reagent (amine) was reduced by 50 percent. Test (c) is the same as (a) except that the amount of positive-ion reagent (amine) was reduced by 75 percent. Test (d) is the comparative run using the conventional mineral acid deactivation and

|                                   | (a)   | (b)   | (c)   |
|-----------------------------------|-------|-------|-------|
| Percent solids in washing step    | 65    | 65    | 40    |
| Pounds reagents/ton concentrates: |       |       |       |
| H <sub>2</sub> SO <sub>4</sub>    | 0.00  | 0.00  | 6.00  |
| Na <sub>2</sub> SiF <sub>6</sub>  | 2.00  | 3.00  | 0.00  |
| NaOH                              | 0.20  | 0.20  | 0.20  |
| Amine                             | 0.20  | 0.20  | 0.20  |
| Frother                           | 0.20  | 0.20  | 0.20  |
| Percent concentrates              | 84.8  | 82.0  | 82.3  |
| Percent silica froth              | 15.2  | 18.0  | 17.7  |
| B. P. L. concentrates             | 77.21 | 76.93 | 77.02 |
| B. P. L. silica froth             | 36.51 | 42.17 | 43.56 |
| SiO <sub>2</sub> concentrates     | 1.42  | 1.31  | 1.40  |
| Percent B. P. L. recovered        | 92.18 | 89.26 | 89.14 |

### Example V

Finally, an additional series of tests was conducted to illustrate the comparative effectiveness of the various fluosilicates. In making these tests, dewatered primary or rougher concentrates were de-reagentized with the various fluosilicates in an amount equivalent to that of sodium fluosilicate. Therefore, the amount used varied with the molecular weight. The rougher concentrates were conditioned with the fluosilicates for two minutes at 65% solids, then washed free of deadened reagents by several decantations with clean water and finally treated with a positive-ion reagent (amine). The results were as follows:

|                               | Na <sub>2</sub> SiF <sub>6</sub> | CaSiF <sub>6</sub> | K <sub>2</sub> SiF <sub>6</sub> | (NH <sub>4</sub> ) <sub>2</sub> SiF <sub>6</sub> | MgSiF <sub>6</sub> |
|-------------------------------|----------------------------------|--------------------|---------------------------------|--------------------------------------------------|--------------------|
| Pounds Reagents/ton Conc.:    |                                  |                    |                                 |                                                  |                    |
| Fluosilicate                  | 2.00                             | 2.31               | 2.16                            | 1.89                                             | 1.76               |
| Amine                         | 0.12                             | 0.12               | 0.12                            | 0.12                                             | 0.12               |
| Pine Oil                      | 0.12                             | 0.12               | 0.12                            | 0.12                                             | 0.12               |
| Metallurgical Results:        |                                  |                    |                                 |                                                  |                    |
| Percent Concentrates          | 90.13                            | 87.82              | 87.43                           | 87.77                                            | 86.65              |
| Percent Silica Froth          | 9.87                             | 12.18              | 12.57                           | 12.23                                            | 13.35              |
| BPL Concentrates              | 78.64                            | 78.81              | 78.88                           | 78.94                                            | 78.57              |
| SiO <sub>2</sub> Concentrates | 1.89                             | 1.84               | 1.60                            | 1.70                                             | 1.66               |
| BPL Silica Froth              | 40.14                            | 44.36              | 47.33                           | 45.34                                            | 48.90              |
| Percent BPL Recovered         | 94.71                            | 92.76              | 92.06                           | 92.55                                            | 91.25              |

These last-described tests indicate that, while all the fluosilicates are applicable, sodium fluosilicate produces slightly superior metallurgical results.

As can be seen from the foregoing examples, the method of the present invention not only provides a valuable use for a hitherto little-used by-product, but it also permits a reduction in the amount of expensive amine reagent required in the silica flotation step without a corresponding reduction in yield or quality of the recovered concentrate. Substantially smaller amounts of these reagents, the fluosilicates, may be used than are required when the conventional sulfuric acid is employed.

The type of flotation reagents, i. e., anionic or cationic, frothers, etc., used in either the initial phosphate float or the subsequent silica float does not form a part of the present invention and is not critical to its operability. Any of the conventional reagents heretofore known may be used in their customary and usual amounts with good success. In obtaining the rougher concentrates used in the above examples, the feeds were treated in the conventional manner with higher fatty acids, caustic soda, and fuel oil.

Obviously, many modifications and variations of the invention as hereinbefore set forth may be made without departing from the spirit and scope thereof, and therefore only such limitations should be imposed as are indicated in the appended claims.

We claim:

1. In a process for concentrating phosphate values from phosphate ore by a reverse flotation process wherein a negative-ion reagent is used to separate a rougher concentrate rich in phosphate and lean in silicious impurities, the negative-ion reagent deactivated and a positive-ion reagent used to separate the silicious impurities from the phosphate, the improvement which comprises treating the rougher concentrate with a water-soluble fluosilicate to deactivate said negative-ion reagent prior to separating the silicious impurities with the positive-ion reagents.

2. The process of claim 1 wherein the fluosilicate is an alkali metal silicate.

3. The process of claim 1 wherein the fluosilicate is an alkaline earth fluosilicate.

4. A process for the concentration of phosphate values from phosphate ore which comprises: subjecting the ore to a flotation operation with negative-ion reagents to float off a rougher concentrate rich in phosphate values and containing small amounts of entrained silicious impurities; conditioning said rougher concentrate with a small amount of a water-soluble metal fluosilicate to destroy the effect of said negative-ion reagents; and thereafter subjecting said rougher concentrate to a further flotation operation with positive-ion reagents whereby said silicious impurities are floated off and a concentrate rich in phosphate values is obtained.

5. A process for the concentration of phosphate values from phosphate ore which comprises: subjecting the ore to a flotation operation in the presence of a higher fatty acid, caustic soda and fuel oil to float off a rougher concentrate rich in phosphate values and containing small amounts of entrained silicious impurities; conditioning said rougher concentrate with a small amount of a water-soluble fluosilicate to destroy the effect of the agents used in its production; and thereafter subjecting said rougher concentrate to a further flotation operation with a positive-ion reagent whereby said silicious impurities are floated off and a concentrate rich in phosphate values is obtained.

6. A process for the concentration of phosphate values from phosphate ore which comprises: subjecting the ore to a flotation operation with a reagent to float off a rougher concentrate rich in phosphate values and containing small amounts of entrained silicious impurities; con-

ditioning said rougher concentrate with a small amount of a water-soluble fluosilicate to destroy the effect of said reagent; washing the said concentrate to remove the reagent so conditioned; and thereafter subjecting said washed rougher concentrate to a further flotation operation with a reagent whereby said silicious impurities are floated off and a concentrate rich in phosphate values is obtained.

7. A process for the concentration of phosphate values from phosphate ore which comprises: subjecting the ore to a flotation operation with a negative-ion reagent to float off a rougher concentrate rich in phosphate values and containing small amounts of entrained silicious impurities; conditioning said rougher concentrate with a small amount of a water-soluble fluosilicate to destroy the effect of said negative-ion reagent; washing the said concentrate to remove the negative-ion reagent so conditioned; and thereafter subjecting said washed rougher concentrate to a further flotation operation with a positive-ion reagent whereby said silicious impurities are floated off and a concentrate rich in phosphate values is obtained.

8. A process for the recovery of phosphate values from phosphate ore which comprises: subjecting the ore to a concentrating operation in the presence of negative-ion reagents whereby a rougher concentrate rich in phosphate values and containing said negative-ion reagents and a small amount of silicious impurities is formed; conditioning said rougher concentrate with a small amount of sodium silico fluoride to destroy the effect of said negative-ion reagents; and thereafter subjecting said rougher concentrate to a further concentrating operation in the presence of positive-ion reagents whereby said siliceous impurities are removed and a concentrate is obtained which is rich in phosphate values.

9. In a reverse flotation process for the recovery of phosphate values from phosphate ore wherein the ore is first subjected to a concentration operation in the presence of negative-ion reagents followed by a second concentration operation in the presence of positive-ion reagents, the improvement which comprises: contacting the ore from the first concentration operation with a small amount of sodium silico fluoride to destroy the effect of the negative-ion reagents prior to subjecting the ore to the second concentration operation.

10. A process for the concentration of phosphate values from phosphate ore which comprises: subjecting the ore to a flotation operation with a reagent to float off a rougher concentrate rich in phosphate values and containing small amounts of entrained silicious impurities; conditioning said rougher concentrate with a small amount of a water-soluble fluosilicate to destroy the effect of said reagent; and thereafter subjecting said rougher concentrate to a further flotation operation with a reagent whereby said silicious impurities are floated off and a rougher concentrate rich in phosphate values is obtained.

11. The process of claim 10 wherein the fluosilicate is sodium fluosilicate.

12. The process of claim 10 wherein the fluosilicate is calcium fluosilicate.

13. The process of claim 10 wherein the fluosilicate is potassium fluosilicate.

14. The process of claim 10 wherein the fluosilicate is ammonium fluosilicate.

15. The process of claim 10 wherein the fluosilicate is magnesium fluosilicate.

#### References Cited in the file of this patent

#### UNITED STATES PATENTS

2,414,815 Kennedy et al. Jan. 28, 1947  
2,469,422 Weinig May 10, 1949